

Oct. 3, 1950

R. D. GREEN

2,524,439

METHOD AND APPARATUS FOR TREATING WIRE PRODUCTS

Filed Dec. 31, 1946

2 Sheets-Sheet 1



INVENTOR  
RICHARD DUANE GREEN

BY  
Philip Churchill  
ATTORNEY

Oct. 3, 1950

R. D. GREEN

2,524,439

METHOD AND APPARATUS FOR TREATING WIRE PRODUCTS

Filed Dec. 31, 1946

2 Sheets-Sheet 2

Fig. 5.



Fig. 4.



## UNITED STATES PATENT OFFICE

2,524,439

METHOD AND APPARATUS FOR TREATING  
WIRE PRODUCTS

Richard Duane Green, Trenton, N. J., assignor to  
John A. Roebling's Sons Company, Trenton,  
N. J., a corporation of New Jersey

Application December 31, 1946, Serial No. 719,420

11 Claims. (Cl. 57—55.5)

1

This invention relates to the treatment of wire rope, strand, cable and the like to improve the physical properties of such products, and more particularly relates to a method and apparatus for treating such products under tension.

Various procedures have been suggested heretofore for pre-stretching wire rope and particularly wire rope designed for uses such as elevator cables. Although some rather exaggerated claims have been made, such procedures as have been adopted heretofore have attempted to remove what is known as the constructional stretch from the rope, or, in other words, to produce an elongation of the rope approximately equal to that which takes place after an untreated rope has been in actual use for some time.

Such treatments by the application of tension alone have had little or no effect on other physical properties of the rope such as its fatigue resistance and its ultimate strength. Also, such treatments have involved either expensive extra equipment, or extra equipment plus an entirely separate operation, with an attendant substantial increase in the cost of manufacturing the rope.

One object of this invention is to provide a treatment for wire strand, cable, rope and the like which is simple and relatively inexpensive to perform and which produces many improvements in the physical properties of the product.

Another object is the provision of a method and apparatus for improving the physical properties of such materials by subjecting them under controlled conditions to tension in excess of the proportional limit of the material being treated.

A further object of the invention is the provision of method and apparatus for treating such materials by flexing them under tension in such a manner that at least a majority of the individual wires of the product are stretched sufficiently to produce permanent set.

Another object of this invention is the provision of method and apparatus for treating wire rope, and particularly lang lay wire rope, by subjecting it to a high degree of tension while the rope is on a pull-out mechanism serving to pull the wire rope through the closing die.

A further object is to manufacture wire rope, strand, cable and the like by substituting for an ordinary pull-out mechanism in the stranding or closing machine, a pull-out in which the drums have portions of different diameters to subject the product to the required amount of tension.

Other objects and advantages will be explained and will be apparent from the following description of the invention in connection with the drawings, in which:

2

Fig. 1 is a somewhat diagrammatic side elevational view of a special pull-out mechanism in accordance with this invention associated with a closing die and take-up reel.

Fig. 2 is a top plan view of the apparatus shown in Fig. 1.

Fig. 3 is a radial sectional view on a still larger scale taken through the outer portion of one of the differential diameter drums in the pull-out mechanism shown in Fig. 3.

Fig. 4 is a fragmentary plan view of the tensioning mechanism on a larger scale than Fig. 1 to show the manner in which a wire rope is subjected to tension and flexing.

Fig. 5 is a fragmentary longitudinal sectional view on a larger scale through the tensioning mechanism.

In accordance with my invention a structure composed of individual wires twisted together, such as wire strand, cable, rope and the like, is subjected to a high degree of tension and preferably a tension high enough to produce an actual permanent set in most, if not all, of the individual wires making up the structure.

While the structure is under this tension, it is preferably subjected to repeated flexing or working. For best results, the amount of tension should be in excess of the proportional limit of the product being treated, and preferably in excess of 70% of the ultimate or breaking strength of such product. For practical purposes, the proportional limit of the product treated may be considered to be the unit stress on a stress-strain diagram at which the rate of deformation is 50% greater than the minimum rate of deformation.

I have found that such a high degree of tension, particularly when it is accompanied by flexing or working under tension, produces very beneficial improvements in the physical properties of the structure. It is apparent, of course, that such a treatment removes what is known as the constructional stretch or, in other words,

that part of the elongation which results from the compacting of the structure of a wire rope or strand. In addition to removing the constructional stretch, however, this treatment, particularly as applied in accordance with the procedure I prefer as described below, produces a final product that has a substantially higher fatigue resistance; that has a somewhat higher ultimate strength; and that is extremely uniform in its properties throughout its entire length.

Such uniformity makes it much easier to predict what a long length of strand or rope will do in actual performance since much greater reliance can be placed upon results obtained from physical tests of a short length of the material.

My invention has still further advantages when applied to the treatment of particular products such as lang lay rope, a material that is very difficult and expensive to make satisfactorily. At present, the manufacture of high quality lang lay rope requires special precautions in its manufacture, such as the use of special stranding and closing machines to put back-twist into the individual wires as the strand is made, or to regulate carefully the twist that is given to the strands as they are fed to a closing die in a closing machine. For most purposes, stranding and closing machines that operate at relatively slow speeds must be used in order to produce a high quality lang lay rope, and such procedures all add to its cost.

The process of my invention may be applied to a finished lang lay rope made without taking these special precautions and makes it possible to produce a high quality lang lay rope that is even less cranky than usual, as well as having the other improved properties mentioned above. This is particularly important economically because the process of my invention may be applied, particularly in its preferred form, to the manufacture of wire rope without using any additional step or extra equipment in the entire process.

The preferred apparatus for carrying out my invention is illustrated in the drawings as applied, for example to the manufacture of wire rope. The strands 10 in a closing machine are fed in any suitable manner to a closing die 11. Instead of using the customary pull-out mechanism to pull the wire rope 12 through the closing die, I employ a pair of drums 13 and 14 spaced from each other in the usual manner but having on each drum, sections 15 of one diameter and sections 16 of a larger diameter. These drums may be mounted upon suitable shafts 17 and 18 and driven through gears 19 and 20 by means of the small pinion gear 21 associated with the motor 22. As will be apparent, any source of power may be used to drive these drums so that they are rotated in the same direction at the same speed. If desired, the bearings 23, 24 for the shafts 17 and 18 respectively may be rigidly held apart by an adjustable bar or rod 25.

The wire rope 12 from the closing die 11 is passed for several wraps or turns around the smaller diameter sections 15 of the two drums 13 and 14. In accordance with well known practice, the sections 15 and 16 of these drums are preferably provided with annular grooves 26 of proper diameter to receive the wire rope 12.

The wire rope then passes from the last groove in the sections 15 to the first groove in the sections 16 and may then be passed for several turns around the larger diameter sections 16 of the two drums. The rope moves from the drums 13 and 14 to a take-up reel 27 mounted on a suitable standard 28 and preferably driven by a motor or other means (not shown) connected to the shaft 29.

It will be apparent that the grooves in the larger diameter sections 16 of the two drums travel at a higher peripheral speed than the grooves in the smaller diameter sections 15. Thus, in a given number of rotations, the rope on the drum sections 16 will be traveling a greater distance than the rope on the drum sections 15. This creates a high degree of tension in the rope on the two drums. As a practical

matter, the drums can be arranged with the proper differential in diameters between the sections 15 and 16 and the proper number of wraps or turns of the rope about each section to produce any desired degree of tension in the rope.

It has been found that the tension of the rope on the smaller sections 15 increases as the rope gets closer to the inside groove from which it transfers to the first groove on the larger diameter sections 16. The peak tension is applied to the rope passing from the last groove in the smaller diameter section 15 to the first groove in the larger diameter section 16. Thereafter, the tension in each successive turn of the rope around the larger diameter sections 16 decreases until the point is reached at which the rope passes to the take-up reel. A certain amount of slippage as well as creepage of the rope on the drums takes place which accounts for this tension variation.

If relatively few turns of the rope are used about each of the sections of the differential diameter drums, it may be desirable to have a greater take-up tension applied by the reel 27 than would normally be used. This is needed to prevent undue slippage which might result in the application of a much lower peak tension to the rope than is desired. For most practical purposes, the back tension applied by the closing die 11 is entirely adequate to prevent undue slippage of the rope on the smaller diameter sections 15.

Care must be exercised in choosing the diameters to be used for the sections 15 and 16 and in the selection of the number of turns or wraps about each section of the drum, as well as in the amounts of back tension applied to the rope on the drums to provide sufficient tension but still avoid the application of such a high tension as will produce failure or rupturing of the rope. The rope is also being flexed repeatedly while it is under tension by reason of its passage along successively straight and curved paths. This flexing produces a very beneficial actual working of the rope or similar structure as well as of the materials comprising the structure while they are in the plastic range, i. e., under a tension in excess of the proportional limit.

It will be seen that the differential pull-out mechanism of my invention may be very simply substituted for an ordinary pull-out mechanism customarily used on a stranding or closing machine, so that the use of my invention does not actually involve additional apparatus, but does supply an additional and very beneficial processing of the product being treated. From the economic point of view, the strand, cable or rope may be made in accordance with my invention at low cost without the necessity of using either special preliminary treatments or expensive after treatments of the product. At the same time, the final product, probably because of the manner in which it is subjected to the tension as well as the amount of tension applied, has its physical properties improved to a very surprising degree.

While one form of the invention has been described in connection with the example illustrated in the drawings, it will be apparent to those skilled in the art that many variations may be made in the apparatus as long as the product is subjected to the proper amount of tension alone or to a combination of such tension with flexing or working to produce the desired improvements in physical properties.

I claim:

1. A process of treating wire strand or rope to increase its ultimate strength which comprises moving such material longitudinally and subjecting successive short lengths of the moving material to tension that is increased to a maximum and then reduced, the maximum tension being substantially in excess of the proportional limit of the material so that permanent set is imparted to at least a majority of the individual wires in said material.

2. A process of treating wire strand or rope to produce a greater resistance to fatigue and higher ultimate strength which comprises moving such material alternately through straight and curved paths and subjecting successive short lengths of the moving material for short periods of time to tension of at least about 70% of the ultimate strength of the material but less than said ultimate strength.

3. A process of treating wire rope to improve its uniformity and increase its strength after fatigue by flexing the rope while under tension which comprises moving said rope through a plurality of alternate straight and curved paths, increasing the tension on such rope at successive straight paths until a maximum tension is reached, and thereafter relieving said tension, said maximum tension being substantially higher than the proportional limit for said rope.

4. A process of treating lang lay wire rope to increase its strength after fatigue and ultimate strength which comprises moving said rope through a plurality of alternate straight and curved paths, increasing the tension on such rope at successive straight paths until a maximum tension is reached, and thereafter relieving said tension gradually in successive stages, said maximum tension being substantially higher than the proportional limit for said rope.

5. In a process of making wire strand, wire rope and the like, the steps of passing the material around a plurality of driven drums having cylindrical portions of different diameters, moving the material after several turns from the smaller diameter portions of said drums to the largest diameter portions thereof, and maintaining tension on the material issuing from said drums, the difference in diameters of said portions and said issuing tension being sufficient to apply a maximum tension above the proportional limit of the material but insufficient to rupture the material.

6. In apparatus for making wire strand, rope and the like, a pull-out device comprising a pair of capstans having portions to receive the product from a forming die, and other portions opposite each other traveling at a higher peripheral speed that receive the product from said first mentioned portions whereby the product is subjected to increased tension as it passes to said second mentioned portions.

7. In apparatus for making wire strand, rope and the like, a pull-out device comprising a pair of drums, each drum having cylindrical portions of different diameter, and means for rotating said drums at the same speed in the same direction, said portions of smaller diameter being arranged to receive the product from a forming die and said portions of larger diameter being arranged to receive the product from said portions of smaller diameter whereby the product is subjected to tension which reaches a maximum as the product moves from said smaller to said larger diameter portion.

8. Apparatus for treating a twisted wire product to improve its physical properties which comprises a pair of drums arranged to rotate in the same direction on axes parallel to each other, each drum having cylindrical portions opposite each other of smaller diameter and cylindrical portions opposite each other of larger diameter, each of said portions being of sufficient size to apply several wraps of the product thereon, means for supplying the product under back tension to said smaller diameter portions, and means to maintain sufficient tension on the product issuing from said larger diameter portions to prevent undue slippage of the product on the drums, the difference in diameter of said portions being sufficient to create tension in the product above its proportional limit but below its breaking limit.

9. In apparatus for making wire strand, wire rope and similar twisted wire products, the combination of a closing die for forming the twisted product, and a pull-out device for pulling the product through said die and simultaneously stretching the product which comprises a pair of drums rotating about substantially parallel axes having opposed cylindrical portions of different effective diameters arranged so that the smaller diameter portions receive the product from said die and the larger diameter portions receive the product from said smaller diameter portions, and means for driving said drums.

10. A process of making wire rope having an increased strength after fatigue which comprises forming the rope and immediately thereafter passing the rope around a pair of drums rotating at the same speed and each drum having cylindrical portions of different diameters, the rope passing first around the portions of smaller diameter and then around the portions of larger diameter, and maintaining tension on the rope as it leaves the drums, the difference in diameters between said portions and the tension on the rope passing to and leaving the drums being sufficient to subject the rope to a maximum tension of at least 70% of the ultimate strength of the rope but less than its breaking strength.

11. In apparatus for making wire rope, a pull-out device comprising a pair of capstans each of which has a generally cylindrical portion of smaller and an adjacent generally cylindrical portion of larger diameter, the smaller and larger diameter portions of the two drums being opposite each other and disposed so that rope from a closing die passes first around the smaller diameter portions and thence around the larger diameter portions whereby the rope is subjected to tension that is substantially increased while the rope is on the capstans, and means for driving said capstans in the same direction at the same speed.

RICHARD DUANE GREEN.

#### REFERENCES CITED

The following references are of record in the 65 file of this patent:

#### UNITED STATES PATENTS

| Number    | Name                | Date          |
|-----------|---------------------|---------------|
| 286,258   | Brownell            | Oct. 9, 1883  |
| 1,692,505 | Hoffmann            | Nov. 20, 1928 |
| 1,955,540 | Ellis et al.        | Apr. 17, 1934 |
| 2,087,606 | Oppenlaender et al. | July 20, 1937 |
| 2,372,627 | Goggin et al.       | Mar. 27, 1945 |
| 2,389,878 | Symmes              | Nov. 27, 1945 |